

June 22, 1971

L. B. WILDER ET AL

3,585,710

METHOD OF ATTACHING A CARBIDE RING TO A STEEL TUBE

Filed Dec. 30, 1968



FIG. 1



FIG. 2

INVENTORS  
LAWRENCE B. WILDER  
BY RENIC P. VINCENT

*John S. Gassett*  
ATTORNEY

## 1

3,585,710

### METHOD OF ATTACHING A CARBIDE RING TO A STEEL TUBE

Lawrence B. Wilder and Renic P. Vincent, Tulsa, Okla.,  
assignors to Pan American Petroleum Corporation,  
Tulsa, Okla.

Filed Dec. 30, 1968, Ser. No. 787,909  
Int. Cl. B23k 31/02

U.S. Cl. 29—473.1

5 Claims

#### ABSTRACT OF THE DISCLOSURE

This is a method of attaching a carbide ring to the outside of a steel tube such as a valve stem. It overcomes the problem caused by the difference in thermal coefficient of expansion between carbide and steel. In the preferred embodiment of the method employed, molten brazing compound at a high temperature, e.g., 1,700° F., is melted in the clearance space between the carbide ring and the steel tube. The carbide ring is allowed to cool to about 1,000° F. while the steel tube is kept hot to about 1,500° F. by applying heat to the inside. A steel plug is then placed inside the steel tube adjacent the carbide ring. This steel plug has been sized to have a diameter, at room temperature, equal to that of the inside of the steel tube in its expanded position at 1,000° F. After the plug is inserted, heat is no longer applied and the carbide ring continues to shrink and to displace the excess semi-molten brazing compound. The steel tube also starts contracting until it contacts the plug. The plug which was put into the tube at room temperature, e.g., 80° F., has heat transferred to it from the steel tube and the plug itself starts to increase in size. The steel tube when it contacts the plug will be at least at 1,000° F. and is soft enough to yield easily. As the temperature of the steel plug increases, it continues to expand and causes additional yielding of the steel tube which yields sufficiently so that when it and the carbide ring cool, they do not separate.

#### BACKGROUND OF THE INVENTION

##### (1) Field of the invention

This invention is concerned with a method of fastening carbide to steel. It is particularly concerned with the fastening of a carbide ring to the outside of a steel tube.

##### (2) Setting of the invention

It has been very difficult to fasten carbide rings to the outside of steel tubes. A common method of attaching a carbide ring to the steel tube is to leave a clearance space between the two and fill that with a molten brazing compound. This system may be satisfactory if the service for which the assembly is intended is not severe. However, for hard service this method is not at all satisfactory as the attachment will not stand up. The source of the main problem is that the differences in thermal coefficient of expansion between carbide and steel cause a separation of the brazing material as the assembly cools.

Some success has been made in this as described in our U.S. Pat. 3,372,464. However, that system is not always completely satisfactory. For example, in the method described in that patent, slots are provided in the end of the steel tube. It would be preferred that a better method

## 2

be devised and especially one where it would not be necessary to cut slots.

#### SUMMARY OF THE INVENTION

This is a method of attaching a carbide ring to a steel tube. A molten brazing compound is placed between the carbide ring and the steel tube which, when cooled, is bonded to both the steel tube and the carbide ring. Means are provided to apply heat to the inside of the steel pipe while permitting the outer carbide ring to cool. As the carbide ring cools, it contracts. At the same time, means are provided to force the hot steel tube to yield an amount sufficient to compensate for the otherwise decrease in diameter due to cooling over that decrease in size of the carbide ring. Thus, there is not sufficient differential shrinkage to cause separation of the brazing material.

This process in one embodiment is accomplished, for example, by placing a brazing compound at about 1,700° F. between the carbide ring and the steel tube. The outer carbide ring is allowed to cool to about 1,000° F., for example, while the steel tube is kept at about 1,500° F. by applying heat to the inside of the tube. A properly sized steel plug is used to force the inner steel plug to yield while it is still hot. This plug is sized to have a diameter, at room temperature, e.g., 80° F., equal to the inside diameter of the steel tube at 1,000° F., which is sufficiently hot for the steel to yield easily. After the plug is placed inside the tube, the assembly is permitted to cool. The carbide ring continues to shrink and the steel tube contracts until it contacts the plug. The transfer of heat to the plug causes it to expand. This in turn causes the steel tube to yield. Upon final cooling of the assembly, the steel tube decreases in size about the same amount as, or slightly less than, does the carbide ring.

#### BRIEF DESCRIPTION OF THE DRAWINGS

40 Various objects and a better understanding of the invention can be had from the following discussion taken in conjunction with the drawings in which:

FIG. 1 is a cross sectional view of the end of a steel tube with the carbide ring.

45 FIG. 2 illustrates a drawing of the steel plug which is to be inserted into the steel tube of FIG. 1.

#### DESCRIPTION OF THE PREFERRED EMBODIMENTS

50 Attention is directed to FIG. 1 which shows a steel tube 10 and a carbide ring 12 which is to be attached to the outer wall of the tube 10. Shown between tube 10 and carbide ring 12 is a brazing compound 14. Care should be taken so that the brazing compound is evenly distributed about the tube. FIG. 2 illustrates a steel plug and is indicated by reference numeral 16. The function of the plug will be explained subsequently. The plug 16 is preferably solid steel having approximately the same coefficient of thermal expansion as does tube 10. Plug 16 has three portions: a head portion 18, a tapered lead portion 20 and a center portion 22. The relationship of the dimension of portion 22 to the steel tube 10 will be discussed hereinafter.

Various sizes of the steel and carbide parts are indicated in the drawing and are labeled as follows:

$D_{st}$  is the bore diameter of the steel tube;

$D_{so}$  is the outside diameter of the steel tube where the carbide ring is attached;

$D_{ci}$  is the bore of the carbide ring;

$D_p$  is the diameter of section 22 of the steel plug;

$L$  is the length of the section of the steel tube where the attachment is to be made;

$L_1$  is a corresponding part of the plug and  $L=L_1$ .

The thickness of the wall of the tube at the point where the carbide ring 12 is to be attached is one-half the difference between  $D_{st}$  and  $D_{so}$ . The difference between  $D_{st}$  and  $D_{so}$  is determined by the required strength of the tube. The radial clearance between the carbide ring 12 and the tube 10 is one-half the difference between  $D_{so}$  and  $D_{ci}$ . The difference in these diameters is determined by the required radial clearance space for the brazing compound selected. This is ordinarily between about 0.062" and 0.093". Each of these diameters become larger as heat is applied and become smaller as they cool. The problem is that they change at a different rate. For example, the thermal coefficient of expansion for a carbide ring may be  $3.5 \times 10^{-6}$  and for steel it may be  $7.85 \times 10^{-6}$  for the expected temperature range.

Since upon cooling the steel tube shrinks at a faster rate than does the carbide ring, the annular space containing the molten brazing material expands, thus requiring more material to be added if the space is to be maintained full. It is not believed that this increase in volume offers any problem as long as the brazing material is in liquid form. However, after the brazing material starts to solidify, it becomes porous and, in fact, separates from the carbide ring and the steel tube when room temperature is reached. In fact, we have often found that no bond between the brazing compound and the carbide ring or the steel tube remains after it is cooled.

We have found a system whereby this annular volume or space between the carbide ring and the steel tube can be made to decrease in volume as the assembly cools. Therefore, the brazing material becomes more dense as it is compressed in the annular volume rather than more porous as is the case if the volume increases in size. The process and the means by which the natural physical properties of the materials are used to accomplish this are described below.

The process of this invention has been successfully used to attach a carbide ring such as ring 12 to a steel tube such as tube 10. The brazing material used is identified as "All-State 11," which is commercially available. All surfaces to be attached by brazing, such as the inner surface of the carbide ring 12 and the mating outer surface 15 of the steel tube 10, are first covered with a suitable flux. Then the carbide ring 12, while resting on shoulder 13 of the steel tube, is centered over tube 10. The assembly is in an upright position as indicated in the drawing. By way of explanation, in one successful application, the assembly was heated to 1,700° F. and the molten brazing material was flowed into place in the annular volume or space between the carbide ring 12 and the steel tube 10. At this time heat is applied to the interior portion of tube 10 adjacent the carbide ring by any well known means such as by an oxygen acetylene torch, not shown. At this time no heat is applied to the carbide ring 12 from the outside, but it is allowed to cool.

Heat is continued to be applied to the inside of the steel tube until equilibrium heat flow from the inside of the tube to the carbide ring is reached. The heat applied to the inside of the tube is that necessary to keep the brazing material between the tube 10 and the carbide ring 12 semi-molten. One way this condition can easily be checked is by applying a brazing rod (of the same material as the semi-molten brazing material) at frequent time intervals to the semi-molten brazing material. The temperature should be just

high enough so that the new brazing rod melts. At this temperature the brazing compound in the space between the ring 12 and tube 10 is in the semi-molten stage. This test is possible because the brazing material used has a remelt temperature which is some 20° to 50° F. higher than that for the first melt. This process allows the carbide ring to shrink to its minimum diameter consistent with the average temperature. Some of the brazing material will be displaced due to the reduced annular space which was caused by cooling of the carbide ring while maintaining the steel tube at a higher temperature, e.g., 1,500° F.

At this stage of the process, the heat source for the interior of the tube 10 is removed and the cylindrical surface 22 of plug 16 inserted adjacent the carbide ring 12. Cylindrical surface 22 has been machined so that its diameter  $D_p$  is equal to the diameter of the bore of tube 10 at a temperature at which the steel stem will still yield easily. A suitable temperature is about 1,000 to 1,200° F. As no heat is being applied to tube 10 now, tube 10 will continue to shrink and will contact surface 22 of plug 16. Heat from the assembly flowing through the steel plug causes its diameter  $D_p$  to expand. This expansion causes the bore of tube 10 to be expanded. As carbide ring 12 is also reduced in diameter, this causes a reduction in the annular volume for the brazing material 14. The carbide ring 12 continues to cool and its diameter  $D_{ci}$  decreases, but the plug 16 continues to expand due to its increased temperature resulting from the heat flow from the assembly to the plug. As the plug expands, the tube 10 being at an elevated temperature state yields easily and its diameter is therefore increased. This yield is substantially non-reversible. These actions continue until the plug has reached its maximum temperature and diameter.

After this latter equilibrium temperature is reached, the plug starts cooling and will decrease in diameter. However the steel tube has been forced to yield and will not decrease in diameter, or at least only to a very limited degree, so that there is no appreciable increase in the size of the annular volume occupied by the brazing material. The steel tube has a diameter  $D_{st}$  after cooling which will remain at about the same size as it was when it was at 1,200° F., or whatever the temperature was when heating equilibrium was reached. The plug 16, on the other hand, after it cools, i.e., to about 80° F., will have decreased its diameter sufficiently so that it can easily be removed.

The use of the process just described resulted in a method of fastening a carbide ring to a steel tube which has been found to be permanent. Such an assembly has been operated with the contact force hard enough to break the carbide ring but such force did not disturb the brazed bond.

While the above invention has been described with a great deal of detail, various modifications can be made therefrom without departing from the spirit of the invention.

What we claim is:

1. A method of attaching a carbide ring to the outside of a steel tube which comprises:  
placing said carbide ring around said steel tube;  
placing a molten brazing compound in the clearance between said ring and said tube;  
allowing the carbide ring to cool relative to the temperature of the steel tube while maintaining said steel tube at a temperature at which it yields easily;  
forcing said steel tube to yield radially to have an enlarged diameter; and  
permitting the assembly to cool to ambient temperature.

2. A method as defined in claim 1 in which heat is applied to the inner part of said steel tube after the placing of the brazing compound to maintain the tube at about 1,500° F. while permitting the carbide ring to cool to about 1,000° F.

3. A method as defined in claim 1 in which said step of forcing said steel tube to yield includes placing a steel

plug into said steel tube, which plug at ambient temperature has a diameter equal to the inside diameter of the steel tube when it is at the lowest temperature at which it yields easily.

4. A method of fastening a carbide ring to the outside of a steel tube which comprises the steps of:

placing said ring around said tube;

placing a molten brazing compound between said ring and said tube;

permitting the carbide ring to cool to a temperature between about 1,000° F. and 1,200° F. while applying heat to the inside of said tube to keep it at about 1,500° F.;

10 placing a steel plug which is cool with respect to the tube, into said tube, said plug having a diameter when cool equal to that of the inside of the steel tube at 1,000° F.;

permitting the assembly to cool and thereafter removing the steel plug.

5. A method of attaching a carbide ring to an unslotted 20 steel tube which comprises:

centering the steel tube within the carbide ring to form an annular space;

placing a molten brazing compound in said space; reducing the volume of said space while allowing said carbide ring, said brazing compound and said steel tube to cool by permanently increasing the diameter of said steel tube.

#### References Cited

#### UNITED STATES PATENTS

|           |         |                   |       |          |
|-----------|---------|-------------------|-------|----------|
| 1,403,257 | 1/1922  | Lewis             | ----- | 29—447X  |
| 1,891,304 | 12/1932 | Everett           | ----- | 29—447UX |
| 2,768,433 | 10/1956 | O'Donnell         | ----- | 29—447   |
| 3,050,613 | 8/1962  | Sheinhartz et al. | ----- | 29—447X  |
| 3,298,096 | 1/1967  | Stuart            | ----- | 29—447X  |
| 3,372,462 | 3/1968  | Reid et al.       | ----- | 29—447   |
| 3,372,464 | 3/1968  | Vincent et al.    | ----- | 29—473.1 |
| 3,382,563 | 5/1968  | Barroil et al.    | ----- | 29—447   |

JOHN F. CAMPBELL, Primary Examiner

R. J. SHORE, Assistant Examiner

U.S. CL. X.R.

29—487, 493, 497.5, 507